

# United States Patent [19]

MacKinnon

[11] 4,324,674

[45] Apr. 13, 1982

[54] AMINE SALT STABILIZED PHOSPHATE  
ESTER-BASED FUNCTIONAL FLUID

[75] Inventor: Hugh S. MacKinnon, Hercules, Calif.

[73] Assignee: Chevron Research Company, San  
Francisco, Calif.

[21] Appl. No.: 182,159

[22] Filed: Aug. 28, 1980

[51] Int. Cl.<sup>3</sup> ..... C10M 3/26; C10M 3/28

[52] U.S. Cl. ..... 252/78.5; 252/75;  
252/77; 252/78.1

[58] Field of Search ..... 252/78.5, 78.1, 77,  
252/75

[56]

## References Cited

### U.S. PATENT DOCUMENTS

|           |        |                     |          |
|-----------|--------|---------------------|----------|
| 3,649,721 | 3/1972 | Burrous et al. .... | 252/75 X |
| 3,679,587 | 4/1972 | Smith ....          | 252/75   |
| 3,790,487 | 2/1974 | Burrous ....        | 252/78.5 |
| 3,907,697 | 9/1975 | Burrous ....        | 252/75   |
| 4,206,067 | 6/1980 | MacKinnon ....      | 252/75   |

Primary Examiner—Mayer Weinblatt

Attorney, Agent, or Firm—D. A. Newell; J. J. DeYoung

[57]

## ABSTRACT

The addition of a small amount of a phosphate ester soluble amine salt of a perfluoroalkane sulfonic acid or a perfluoroalkane disulfonic acid to an energy-transmitting functional fluid greatly enhances the anti-erosion properties of the fluid.

8 Claims, No Drawings

## AMINE SALT STABILIZED PHOSPHATE ESTER-BASED FUNCTIONAL FLUID

## BACKGROUND OF THE INVENTION

## 1. Field of the Invention

This invention relates to fluid compositions which are useful for transmitting power in hydraulic systems. Specifically, it relates to power transmission fluids having a tendency to cause erosion of hydraulic systems and a newly discovered means of controlling such erosion.

Organic phosphate ester fluids have been recognized for some time as advantageous for use as the power transmission medium in hydraulic systems. Such systems include recoil mechanisms, fluid-drive power transmissions, and aircraft hydraulic systems. In the latter, phosphate ester fluids find particular utility because of their special properties which include high viscosity index, low pour point, high lubricity, low toxicity, low density and low flammability. Thus, for some years, numerous types of aircraft, particularly commercial jet aircraft, have used phosphate ester fluids in their hydraulic systems. Other power transmission fluid which have been utilized include major or minor amounts of hydrocarbon oils, amides of phosphoric acid, silicate esters, silicones and polyphenyl ethers. Additives which perform special functions such as viscosity index improvement and foam inhibition are also present in these fluids.

The hydraulic systems of a typical modern aircraft contain a fluid reservoir, fluid lines and numerous hydraulic valves which actuate various moving parts of the aircraft such as the wing flaps, ailerons, rudder and landing gear. In order to function as precise control mechanisms, these valves often contain passages or orifices having clearances on the order of a few thousandths of an inch or less through which the hydraulic fluid must pass. In a number of instances, valve orifices have been found to be substantially eroded by the flow of hydraulic fluid. Erosion increases the size of the passage and reduces below tolerable limits the ability of the valve to serve as a precision control device. Many aircraft have experienced sagging wing flaps during landings and takeoffs as a result of valve erosion.

Early investigations indicated that the erosion was being caused by cavitation in the fluid as the fluid passed at high velocity from the high-pressure side to the low-pressure side of the valve. The incorporation of water into the hydraulic fluid was found to inhibit the erosion, but continuing experience shows that a significant erosion problem remains.

Recent studies indicate that certain valve erosions are associated with the electrokinetic streaming current induced by the high-velocity fluid flow.

## 2. Description of the Prior Art

A study of the problem attributing valve erosion to the streaming current induced by fluid flow is Beck et al, "Corrosion of Servovalves by an Electrokinetic Streaming Current", Boeing Scientific Research Document D1-82-0839 (September, 1969) and Beck et al, "Wear of Small Orifice by Streaming Current Driven Corrosion", Transactions of the ASME, Journal of Basic Engineering, Pages 782-791 (December, 1970). Efforts to control hydraulic valve erosion by treating the problem as one of cavitation in the fluid are described in Hampton, "The Problem of Cavitation Erosion In Aircraft Hydraulic Systems", Aircraft Engi-

neering, XXXVIII, No. 12 (December, 1966). The Text, Organophosphorous Compounds, by Kosolapoff (Wiley, New York, 1950), describes methods for preparing organophosphorous derivatives. Several patents describe phosphate ester hydraulic fluids, including U.S. Pat. Nos. 2,636,861, 2,636,862, 2,894,911, 2,903,428, 3,036,012, 3,649,721, 3,679,587, 3,790,487, and 3,907,697.

## SUMMARY OF THE INVENTION

An erosion-inhibited phosphate ester-based functional fluid comprising a major amount of a phosphate ester and from 10 to 50,000 parts per million by weight of a perfluorinated anionic surfactant selected from the group consisting of an amine salt of a perfluoroalkane sulfonic acid or perfluoroalkane disulfonic acid wherein the alkane is from 1 to 18 carbon atoms.

## DETAILED DESCRIPTION OF THE INVENTION

It has been found that by incorporating into a phosphate ester-based functional fluid an effective amount of an amine salt of a perfluorosulfonic acid, the anti-erosion properties of the composition are surprisingly improved.

## Perfluorinated Anionic Surfactant

The perfluorinated anionic surfactants employed in the compositions of this invention are the amine salts of perfluoroalkane sulfonic acids and have the general formula:



where  $R_f$  is a  $C_nF_{2n+1}$  group where  $n$  is an integer of from 1 to 18 or a cyclic  $C_mF_{2m-1}$  group where  $m$  is an integer from 4 to 18,  $x$  is 1 or 2,  $R'$  is a diradical of 2 to 12 carbon atoms, and  $R$  is independently H or an aliphatic, aromatic or heterocyclic group of 1 to 20 carbon atoms, provided at least one  $R$  contains at least one carbon atom, and where 2  $R$  groups may be united to form a heterocyclic group containing 1 or 2 nitrogen atoms. The total number of carbon atoms in all the  $R$  groups is 1 to 60, preferably, 8 to 30. Most preferred are aliphatic  $R$  groups containing 6 to 10 carbon atoms. The amine salt must be soluble in the phosphate ester-based functional fluid.

The amine salts are made by reacting a suitable amine with a perfluoroalkane sulfonic acid or a perfluoroalkane disulfonic acid. Suitable amines include primary, secondary and tertiary amines.

Representative aliphatic amines include primary amines such as octylamine, pentadecylamine, eicosylamine, cyclohexylamine, and 3-oxapentadecylamine. Representative secondary amines include dihexylamine, diundecylamine, dinoaldecylamine, and di(3,6)-dioxadecylamine. Representative tertiary amines include such compounds as tripropylamine, tritetradearylamine, triicosylamine, and di(2-hydroxyethyl)methylamine.

Representative aromatic amines include aniline, 4-butylaniline, 3-octylaniline, dimethylaniline, N-ethyl-2-nonylaniline, 4-phenylbutylamine, and N-methyl-2-phenylhexylamine.

Representative heterocyclic amines include 3-octylpyrrolidine, 3-dodecylmorpholine, piperidine, N-methyl piperidine, triethylenediamine, piperazine, furfurylamine, and pyridine.

Representative polyamines include octamethylenediamine, tetrabutylethylenediamine, tetraethyl-diethylenetriamine, N,N-dimethylhexamethylenediamine, N,N,N',N'-tetramethylethylenediamine, p-phenylenediamine, and m-xylylenediamine.

An effective amount of the perfluorinated anionic surfactant is employed in the functional fluid composition of this invention which can range from as little as 10 parts per million to as much as 50,000 parts per million by weight of the phosphate ester. Preferably, the functional fluid contains at least 100 ppm and more preferably, 200-500 ppm of the perfluorinated anionic surfactant. Amounts greater than 50,000 parts can be employed if soluble in the fluid, however, no commensurate advantages are obtained thereby.

#### Fluid Base

The power transmission fluid of the present invention comprises a fluid base present in major proportion in which the perfluorosulfonate salts and other additives are contained. The fluid base in which the additives of this invention are employed include a wide variety of base materials, such as organic esters of phosphorus acids, mineral oils, synthetic hydrocarbon oils, silicate esters, silicones, carboxylic acid esters, aromatic hydrocarbons and aromatic halides, esters of polyhydric material, aromatic ethers, thioethers, etc.

The phosphate esters which are the preferred base fluid of the present invention have the formula:



wherein R<sup>1</sup>, R<sup>2</sup> and R<sup>3</sup> each represent an alkyl or aryl hydrocarbon group (As used herein, "aryl" includes aryl, alkaryl, and aralkyl structures and "alkyl" includes aliphatic and alicyclic structures.) All three groups may be the same, or all three different, or two groups may be alike and the third different. A typical fluid will contain at least one species of phosphate ester and usually will be a mixture of two or more species of phosphate esters.

The phosphate esters will each have a total carbon content of 3 to 36 carbon atoms. Individual alkyl groups will usually have 1 to 12 carbon atoms, while individual aryl groups will usually have 6 to 12 carbon atoms. Preferred esters contain 12 to 24 total carbon atoms, preferably, alkyl groups, 4 to 6 carbon atoms, and preferred aryl groups, 6 to 9 carbon atoms. The alkyl groups may be straight- or branched-chain, with straight-chain, such as n-butyl, preferred. Similarly, the alkyl substituents in alkylaryl structures may also be straight- or branched-chain. Generic examples of the phosphate esters include trialkyl phosphates, triaryl phosphates and mixed alkylaryl phosphates. Specific examples include trimethyl phosphate, tributyl phosphate, dibutyloctyl phosphate, triphenyl phosphate, phenyl dicresyl phosphate, ethyl diphenyl phosphate, isopropyl diphenyl phosphate, diisopropyl phenyl phosphate, dibutylphenyl phosphate, tricresyl phosphate, etc.

In practice, phosphate ester fluid base generally contains several phosphate esters mixed together. Usually, one particular ester or several closely related esters will predominate. In a preferred type of fluid, the phosphate ester portion contains only trialkyl and triaryl phosphate esters, with the trialkyl phosphate esters predomi-

nating. Typically, the phosphate ester portion of this fluid will consist of 70-99 weight percent, preferably, 80-92 weight percent trialkyl phosphate esters, with the remainder triaryl phosphate esters. The phosphate ester portion is normally 75-95 weight percent of the total fluid and preferably, 85-95 weight percent.

#### Additives

The power transmission fluids of the present invention generally contain a number of additives which in total comprise 5-25 weight percent of the finished fluid. Among these is water, which may be added or often becomes incorporated into the fluid unintentionally. Such incorporation can occur when a hydraulic system is being refilled and is open to the atmosphere, particularly in humid environments. Unintentional incorporation of water may also occur during the manufacturing process of a phosphate fluid. In practice, it is recognized that water will be incorporated into the fluid and steps are taken to control the water content at a level in the range of 0.1-1 weight percent of the whole fluid. It is preferred that the water content be in the range of 0.1-0.8 weight percent and more preferably, 0.2-0.6 weight percent.

Hydrolysis inhibitors to retard corrosion are often added to hydraulic fluids. They include various epoxides such as the glycidyl ethers described in U.S. Pat. No. 2,636,861. Typical epoxide compounds which may be used include glycidyl methyl ether, glycidyl isopropyl ether, styrene oxide, ethylene oxide, and epichlorohydrin. Hydrocarbon sulfides, especially hydrocarbon disulfides, such as dialkyl disulfide, are often used in combination with the epoxide compounds for additional corrosion suppression. Typical hydrocarbon disulfides include benzyl disulfide, butyl disulfide and diisoamyl disulfide. A particularly preferred class of epoxide hydrolysis inhibitors are those containing two linked cyclohexane groups to each of which is fused an epoxide (oxirane) group. Illustrative are those in which the linking structure contains a carboxylic acid ester group or a dioxane ring.

The hydraulic fluid normally contains 2-10 weight percent, preferably, 5-10 weight percent, of one or more viscosity index improving agents such as alkyl styrene polymers, polymerized organic silicones, or preferably, polyisobutylene, or the polymerized alkyl esters of the acrylic acid series, particularly acrylic and methacrylic acid esters. These polymeric materials generally have a number average molecular weight of from about 2,000 to 300,000.

#### Measurements

It has been found that the rate of valve erosion in aircraft hydraulic system valves varies with the electrical streaming potential of the hydraulic fluid passing through the valve. Streaming potential is defined on Pages 4-30 of the Electrical Engineers Handbook, by Pender and Del Mar (New York, Wiley, 1949). It is the EMF created when a liquid is forced by pressure through an orifice and is a function of factors such as the electrical properties and viscosity of the liquid, the applied pressure, and the physical characteristics of the orifice. Since the streaming potential is dependent on several factors, it is found that the streaming potential measurement of a given fluid on a given apparatus at a given time will vary over a small range. For this reason, the ordinary practice is to select as a standard a fluid

which is considered to have acceptable erosive characteristics. Each day the apparatus is calibrated by measuring the streaming potential of the standard fluid and then comparing the streaming potential of the test fluids against this standard. The apparatus used to measure streaming potential is described in detail in the Beck et al report "Wear of Small Orifices by Streaming Current Driven Corrosion", referred to above. Measurements are taken at room temperature with the fluid pressure adjusted to 1,500 psi. For convenience, the streaming potential detected by the apparatus is impressed across a standard 100,000-ohm resistor to obtain a resultant current, which is reported as the "streaming current" or "wall current".

### EXAMPLES

The following examples illustrate the effectiveness of various amine salts of a perfluoroalkane sulfonic acid in controlling the conductivity and wall current of a functional fluid. Conductivities in excess of  $0.3 \times 10^{-6}$  mho/cm are considered satisfactory with conductivities in the range of 0.3 to  $1.3 \times 10^{-6}$  mho/cm being preferred. Wall currents of less than 0.15 microamperes are considered satisfactory with wall currents less than 0.10 microamperes being preferred.

The hydraulic fluid used in all the examples comprises about 72.5 weight percent tributyl phosphate; 11.8 weight percent tri(isopropylphenyl) phosphate; 12.4 weight percent of a polyacrylate viscosity improver; 2.3 weight percent of 2-(3,4-epoxycyclohexyl)-5,5'-spiro(3,4-epoxy)cyclohexane-m-dioxane; 0.5 weight percent dibutyl paracresol; 0.5 weight percent di(octylphenyl)amine; and trace amounts of a foam inhibitor and a dye.

In the following examples, salts were prepared by reacting a trifluoromethane sulfonic acid with an amine, the salt was blended with the hydraulic fluid, and the conductivity and wall current were measured. The results are listed in TABLE I below.

TABLE I

| Amine                 | Concen-<br>tration<br>ppm | Conductivity<br>(mho/cm) $10^{-6}$ | Wall Current<br>amps ( $10^{-6}$ ) |
|-----------------------|---------------------------|------------------------------------|------------------------------------|
| Cation                |                           |                                    |                                    |
| trioctylamine         | 250                       | 0.4                                | 0.03                               |
| tributylamine         | 200                       | 0.5                                | 0.07                               |
| dodecylamine          | 167                       | 0.35                               | 0.11                               |
| tetramethyl guanidine | 130                       | 0.64                               | 0.09                               |
| Quadrol <sup>1</sup>  | 200                       | 0.36                               | 0.07                               |
| 4-azahexadecylamine   | 190                       | 0.43                               | 0.06                               |

<sup>1</sup>N,N,N',N' tetrakis (2-hydroxypropyl) ethylene diamine

What is claimed is:

1. An erosion-inhibited phosphate ester-based functional fluid comprising a major amount of a phosphate ester and from 10 to 50,000 parts per million by weight of a perfluorinated anionic surfactant selected from the soluble amine salts of a perfluoroalkane sulfonic acid or perfluoroalkane disulfonic acid wherein the alkane is from 1 to 18 carbon atoms.
- 15 2. The composition of claim 1 wherein said salt is the salt of an aliphatic amine containing 8 to 30 carbon atoms.
- 20 3. The composition of claim 1 wherein said salt is the salt of trioctyl amine trifluoromethane sulfonic acid.
- 25 4. The composition of claim 1, in which the phosphate ester is a mixed alkylaryl phosphate.
- 25 5. The composition of claim 1, in which the phosphate ester is a mixture of trialkyl phosphate and triaryl phosphate.
- 30 6. The composition of claim 5, in which the trialkyl phosphate is tributyl phosphate and the triaryl phosphate is tris cresyl phosphate or triisopropylphenyl phosphate.
- 35 7. The composition of claim 3 wherein said fluid contains 200 to 5,000 parts per million of said surfactant.
- 40 8. In a method of operating a hydraulic device wherein a displacing force is transmitted to a displacing member by means of a functional fluid, the improvement which comprises employing as said fluid the composition of claims 1, 2, 3, 6 or 7.

\* \* \* \* \*